

## UNITED STATES PATENT OFFICE

2,686,713

## SULFATE PROCESS TALL OIL AS A RUST INHIBITOR FOR FUEL FRACTIONS OF MINERAL OIL

Ralph V. White, Pitman, Phillip S. Landis, Mickleton, and Elwood B. Backensto, Woodbury, N. J., assignors to Socony-Vacuum Oil Company, Incorporated, a corporation of New York

No Drawing. Application December 9, 1950,  
Serial No. 200,104

7 Claims. (Cl. 44—62)

1

The present invention relates to the prevention of the formation of rust on metallic surfaces in contact with mineral oil products and more particularly to prevention of a formation of rust on metallic surfaces in contact with mineral oil products such as gasoline, naphthas and burning oils.

The problem of preventing the formation of rust on metallic surfaces in contact with mineral oil products has received considerable attention in the past decade with respect to those fractions of mineral oil which are used for lubricating purposes. However, the prevention of the formation of rust on metallic surfaces in contact with what may be termed "light products"; i. e., gasoline, naphtha and burning oils, has not received so much consideration. While the problem may seem to be the same, nevertheless the problem of preventing the formation of rust on metallic surfaces in contact with gasoline, naphthas and the like presents factors which are not encountered when confronted with the problem of preventing the formation of rust on metallic surfaces in contact with lubricating cuts of mineral oil.

One of the most important limitations upon the use of a rust preventive in gasoline, for example, is the limitation that the color of the product must be the same as that of the unprotected gasoline; i. e., the rust preventive must not cause a color change in the gasoline by reaction with the hydrocarbon constituents of the gasoline, dyes, components of tetraethyl lead fluid, ant-oxidants, etc., normally contained or added to gasolines. Furthermore, the rust inhibitor must be one which has no appreciable effect upon the octane rating or any of the other specifications under which the gasoline is sold.

Another factor which is of relatively no importance when considering the formulation of a lubricating oil is that of the effect of extreme pressures on the separation or other action of the rust preventive. Thus, for example, it is well known that products such as gasoline, naphtha and burning oils are in many instances transferred from the refinery to distributing points via pipe lines. Pressures as high as 1200 p. s. i. may be encountered in such pipe line transportation. Consequently, it is essential that the rust preventive remain with the petroleum cut regardless of the pressure to which the cut is subjected.

Another factor controlling the selection of a rust preventive for mineral oil fractions other than lubricating oil fractions is the tendency of some known rust preventives to cause the formation of emulsions. Rust preventives which tend

2

to emulsify the water present with the mineral oil fraction are not useful because they tend to hold unusually large amounts of water in the petroleum products.

Indicative of the problem presented in preventing the formation of rust on metallic surfaces in contact with gasoline, naphtha, burning oils and the like is the fact that 110 materials were tested and failed. Of the 110 that failed, failure 10 was due to a color change in the gasoline in 36 instances. Of the remaining 74, 15 failed because of their tendency to form emulsions and the remainder failed to provide the required protection at practical concentrations. Thus, it is 15 manifest that although a large amount of information has been obtained upon the solution of the problem of preventing the formation of rust on metallic surfaces in contact with lubricating fractions of mineral oil, nevertheless the problem 20 of preventing the formation of rust on metallic surfaces in contact with gasoline, naphthas, burning oils and the like still remains to be solved.

An important limitation upon the use of a rust preventive in gasoline is its effect upon gum formation. As a generalization it can be said 25 that rust preventives are non-volatile in nature and increase the amount of gum formed by the amount of rust preventive added. Consequently, a rust preventive useful in gasoline is one which 30 is effective in concentrations not more than about 0.008 weight per cent of non-volatile residue. Accordingly, it is an object of the present invention to provide a gasoline, naphtha or burning oil fraction of mineral oil containing an amount 35 of rust preventive not substantially in excess of about 0.008 weight per cent non-volatile residue. It has now been discovered that crude "tall oil," deodorized "tall oil," solvent refined "tall oil," polymerized "tall oil" and other available 40 "tall oils" are materials which satisfy all of the requirements of a rust preventive for gasoline, naphthas, burning oils and the like.

"Tall oil" is the name by which a mixture of 45 saturated and unsaturated fatty acids and rosin acids is known to the paper pulp manufacturers. When pulping wood by the sulfate, as distinguished from the sulfite, method the pulping liquor soon becomes contaminated with a soap which can be recovered by acidulating the liquors and skimming the water-insoluble organic material from the liquor. These skimmings of the acidulated liquors are known to the paper pulp manufacturer as tall oil, also spelled talloel, taloil and talol.

A number of materials are available to in-



eral oil such as gasoline, naphthas, burning oils and the like.

We claim:

1. A liquid fuel fraction of mineral oil containing from about 0.00003 per cent to about 0.008 weight per cent of sulfate process tall oil.

2. A liquid fuel fraction of mineral oil containing an amount not exceeding about 0.008 weight per cent of sulfate process tall oil effective to prevent rusting.

3. Gasoline containing an amount not exceeding 0.006 per cent of sulfate process tall oil effective to prevent rusting.

4. Kerosine containing an amount not exceeding 0.006 per cent of sulfate process tall oil effective to prevent rusting.

5. Diesel fuel containing an amount not exceeding 0.006 per cent of sulfate process tall oil effective to prevent rusting.

6. Fuel oil containing an amount not exceeding 0.006 per cent of sulfate process tall oil effective to prevent rusting.

7. Naphtha containing an amount not exceeding 0.006 per cent of sulfate process tall oil effective to prevent rusting.

References Cited in the file of this patent

UNITED STATES PATENTS

|    | Number    | Name           | Date          |
|----|-----------|----------------|---------------|
| 10 | 1,752,145 | Calcott et al. | Mar. 25, 1930 |
|    | 2,281,676 | Cook           | May 5, 1942   |
|    | 2,292,352 | Cook et al.    | Aug. 11, 1942 |
| 15 | 2,431,737 | Davis et al.   | Dec. 2, 1947  |

FOREIGN PATENTS

| Number  | Country | Date         |
|---------|---------|--------------|
| 586,651 | France  | Apr. 1, 1925 |